

Nov. 16, 1926.

1,607,475

P. OTTO

MANUFACTURE OF SEAMLESS TUBING

Filed August 31, 1925

3 Sheets-Sheet 1



Fig. 1.

INVENTOR

Peter Otto

By Byrnes, Stetson, Pardee  
his attorneys

Nov. 16, 1926.

1,607,475

P. OTTO

## MANUFACTURE OF SEAMLESS TUBING

Filed August 31, 1925

3 Sheets-Sheet 2

Fig. 2.



## INVENTOR

Peter Otto

by  
Paynes, Stelling, Parmelee  
his attorneys

Nov. 16, 1926.

1,607,475

P. OTTO

MANUFACTURE OF SEAMLESS TUBING

Filed August 31, 1925 3 Sheets-Sheet 3



INVENTOR

Peter Otto

By *John H. K. Koenig*  
*Attala, St. Louis, Mo.*  
*an attorney*

Patented Nov. 16, 1926.

1,607,475

# UNITED STATES PATENT OFFICE.

PETER OTTO, OF DUSSELDORF, GERMANY, ASSIGNOR TO THE YOUNGSTOWN SHEET AND TUBE COMPANY, OF YOUNGSTOWN, OHIO, A CORPORATION OF OHIO.

## MANUFACTURE OF SEAMLESS TUBING.

Application filed August 31, 1925, Serial No. 53,547, and in Germany July 8, 1924.

Seamless tubes have heretofore been produced by first forming a hollow body by means of a piercing mill and thereafter converting the hollow body into the desired tube. The exceedingly high straining of the material in the rolling from the solid into the hollow cross section causes the finished tube to show laminations and chips, which should not occur if higher requirements are asked of the tubes as regards tensile strength, uniformity and exactness, as in that case there would be a relatively large waste of material, labor and time and also a relatively large consumption of power.

The method of forming a hole in the work piece by means of a mandrel is also objectionable when the tube is required to meet certain rigid conditions. This is because the material is subjected to such a large amount of work during the tube formation and because certain portions of the blank are necessarily displaced in a considerable amount. The piercing process therefore has the disadvantage that unless the operation is held within favorable limits the tubes is damaged.

Casting the original ingot hollow in a sand mold has also been found very unsatisfactory as it leads to irregularities. Each ingot could not be cast separate as the waste due to discarding of the heads was much too large. If ingots of sufficient length to be cut up into a number of work pieces were cast, the structure thereof varied according as to whether the separate work pieces were taken from the lower part of the casting or more towards the top where the blow hole is situated. It was impossible to cast the tubular ingots in a horizontal position by reason of the non-uniformity of the material as regards compactness and purity in the various layers throughout the section. Moreover, there was always the danger that the tubular ingots would contain inclosures of molding sand, especially on their inside wall, which could not be detected, but which would render the rolled tubes unfit for the best service.

I have discovered that all of the above objectionable features of the methods heretofore employed are overcome by producing the initial hollow work piece by the method of centrifugal casting. By centrifugal casting, a tubular ingot can be cast horizontally or substantially horizontally, which is of substantially the same uniformity along its whole length, and which does not exhibit the irregularities which occur in the section of a casting made at rest. Particles of slag can only adhere to the inner side of the hollow body as the centrifugal action throws the specifically heavier metal outwards and the lighter slag is forced towards the interior. There is nothing to prevent constructing the initial ingot of such diameter that the further treatment thereof can be effected without the considerable straining of the material as in the case of the other processes above referred to. The use of the centrifugal casting process for making the hollow initial work piece for the rolling of seamless tubes therefore shows advantages hitherto not thought of, which are made manifest not only by the cheapness of manufacture in itself but also by the avoidance of waste.

Another advantage of this novel process which is of great importance is due to the fact that the casting heat contained within the hollow work piece can be utilized direct. This was hitherto not possible with the casting in sand molds. In the centrifugal casting process, however, the conditions are quite different, as in the centrifugal casting process the casting obtained is ready at once for the rolling steps, without further treatment, whereas in the process of casting in sand molds it is necessary to cut off the discarded heads, casting funnels and the like before the hollow bodies can be conveyed to the rolling devices. By reason of the necessity of subjecting the hollow work pieces obtained by other casting methods to an after treatment and to a thorough control, before they can be conveyed to the rolling devices, a utilization of the casting heat is out of the question. It will be apparent, however, that this can be done very well in the new process, as the hollow body obtained by casting represents a purely tubular form without any projection, and as slag formation on the inside will be removed automatically in the further treatment of the same.

The process may also be improved by passing the centrifugally cast hollow body through a chamber which is protected from being cooled in any suitable manner and in which the hollow body may remain until it can or is to be introduced into the rolling mechanism. This would be of particular advantage if interruptions in the rolling

work should occur and it also may be utilized for heating the hollow body uniformly throughout or for imparting thereto a different temperature or chemical or physical properties other than those which it obtains from the casting process, particularly with regard to the required various tensile strengths of the tubes to be produced.

It also may be necessary for the rolling process to be carried out at a considerably lower temperature than that possessed by the hollow body when it leaves the mold. It would be necessary to cool the hollow body either by allowing it to remain for some time exposed to the air, before it is subjected to the rolling process, or it could be cooled artificially.

According to the present invention therefore the centrifugal casting process is used only for the production of comparatively short hollow initial ingots which are further treated by a rolling process until a tube of the required dimensions is obtained. In its simplest form, the invention contemplates passing the hollow ingot directly from the casting mold into the rolling mill.

Suitable apparatus for carrying out the process is shown in the accompanying drawings, wherein:

Figure 1 is a view partly in section and partly in elevation of apparatus for the centrifugal casting of the hollow ingots;

Figure 2 is a similar view of a modified form of such apparatus;

Figure 3 is a sectional view of one form of roughing mill;

Figure 4 is a view of another form of roughing mill; and

Figure 5 is a sectional view of a pilger mill which may be used as the finishing mill.

Referring to the construction shown in Figure 1, the casting device comprises a mold 2 closed at its lower end by a cover 3 to such an extent that the material which is introduced into the mold cannot flow out. The mold is rotatably mounted in bearings 4 and is adapted to be rotated by gears 5 and 6. At the inlet side of the mold is provided a casting truck 7 which receives the molten metal from the casting ladle 8. At the other side of the mold there may be provided any suitable form of conveying device for conveying the cast body 9 to a rolling mill. This conveying device may carry the hollow body into a chamber of the character referred to above for the purpose of regulating the temperature of the cast ingot as explained.

The casting of the hollow body is effected in such a manner that the molten metal supplied to the rotating mold is uniformly distributed over the required length of the mold by suitably moving the casting truck 7 so that a hollow body having walls of sub-

stantially uniform thickness is obtained. After the casting has been completed the cover 3 is removed so that on further rotation of the mold the hollow body slides out of it and is received by the conveying device referred to.

Figure 2 shows casting apparatus very similar to that shown in Figure 1. In the construction shown in this figure, the mold 10 is rotatably mounted in bearings 11 supported by a truck 12. The mold is rotated by a shaft 13 through the pinion 14 and ring gear 15. The liquid metal is supplied from the casting ladle 16 from which it runs through a channel 17 into the rotating mold. By moving the truck 12 the metal can be uniformly distributed in the mold chamber to produce a hollow body having walls of substantially uniform thickness.

After the hollow ingot 9 has been obtained in the manner described, it may be passed to a roughing mill consisting of a pair of grooved rolls 18 and a mandrel 19, such as shown in Figure 3 or it may be passed to a roughing mill of the Mannesman type, such as shown in Figure 4, consisting of the pair of rolls 20 and the mandrel 21. In this preliminary rolling in the roughing mill, the hollow ingot obtained by the centrifugal casting may be only compressed to such an extent as to smooth the walls of the same and to remove the slag or this preliminary rolling process can be used for the purpose of obtaining such variations of diameter as are desirable for carrying out a smooth finishing rolling operation.

The finishing rolling operation is preferably carried out in a pilger mill which is shown in Figure 5. This mill comprises a pair of pilger rolls 22. Each of these rolls has a groove 23 extending part way around the same, the rolls being cut away between the ends of the grooves, as indicated by the reference numeral 24. The hollow ingot 25 received from the roughing mill is supported on a mandrel 26 and the ingot and mandrel are yieldingly forced in the direction of the arrow 27 between the rolls by fluid pressure means (not shown). The rolls rotate in the direction of the arrows 28, and thereby tend to force the ingot and mandrel backwardly in a direction counter to the direction in which they are moved by the fluid pressure means. The rolls are shown with their grooved portions biting into an unreduced portion of the ingot. As the rolls continue to rotate this unreduced portion is rolled down to the thin wall of the tube and when the cut away portions 24 come opposite each other another unreduced portion of the ingot is moved between the rolls to be acted upon by the grooved portions in the same manner.

While I have shown and described certain preferred forms of apparatus for car-

rying out my new process, it will be understood that the invention is not limited to the particular devices shown. For example the finishing rolling may be done by an automatic mill or by a continuous tube rolling mill instead of by a pilger mill such as shown.

I claim:

1. In the manufacture of seamless rolled tubes, the steps consisting in forming an initial hollow ingot by centrifugal casting and thereafter rolling the ingot so formed into the desired seamless tube while utilizing the casting heat contained within the hollow ingot in the rolling, substantially as described.
2. In the manufacture of seamless rolled tubes, the steps consisting in producing an initial hollow ingot by centrifugal casting, passing the ingot so produced through a chamber wherein the ingot is brought to the desired temperature condition, and thereafter rolling the ingot into the desired tube, substantially as described.
3. In the manufacture of seamless tubes, the steps consisting in forming an initial body by centrifugal casting, the body being in the form of an uninterrupted ring at any cross-section thereof, and passing the body in such form lengthwise through a tube mill in the ordinary manner to produce a seamless tube, substantially as described.
4. In the manufacture of seamless tubes, the steps consisting in forming an initial

body by centrifugal casting, the body being in the form of an uninterrupted ring at any cross-section thereof, and, before the body has become cold, passing it in such form lengthwise through a tube mill in the ordinary manner to produce a seamless tube, substantially as described.

5. In the manufacture of seamless tubes, the steps consisting in forming an initial body by centrifugal casting, artificially varying the temperature of the blank thus produced from the temperature which it possesses due to the casting step, the body being in the form of an uninterrupted ring at any cross-section thereof, and passing the body in such form lengthwise through a tube mill in the ordinary manner to produce a seamless tube, substantially as described.

6. In the manufacture of seamless tubes, the steps consisting in introducing molten metal to an elongated centrifugal mold so as to cast a hollow body, shifting the point of introduction of the molten metal during the casting operation, the cast hollow body thus produced being in the form of an uninterrupted ring at any cross-section thereof, and passing the body in such form lengthwise through a tube mill in the ordinary manner to produce a seamless tube, substantially as described.

In testimony whereof I have hereunto set my hand.

PETER OTTO.